

## UNITED STATES PATENT OFFICE

ERICH TRECKMANN AND BRUNO TRECKMANN, OF BERLIN-TEMPELHOF, GERMANY, ASSIGNORS, BY MESNE ASSIGNMENTS, TO LUFTSCHIFFBAU ZEPPELIN, GESELLSCHAFT MIT BESCHRANKTER HAFTUNG, OF FRIEDRICHSHAFEN, BODENSEE, GERMANY

## COMPOSITION FOR IMPREGNATING BALLOON FABRICS

No Drawing. Application filed August 27, 1921, Serial No. 495,935, and in Germany March 3, 1916.

(GRANTED UNDER THE PROVISIONS OF THE ACT OF MARCH 3, 1921, 41 STAT. L. 1313)

Our invention refers to the manufacture of balloon envelope material and more especially to an adhesive and impregnating mass for use in such manufacture. Its particular object is to produce, by aid of the said mass, a balloon envelope material of lighter weight and at the same time to obtain a saving in material as compared with the methods of manufacture carried on until now.

10 The material used up to date in the manufacture of balloon envelopes consisted either of waterproofed cloth or of goldbeater's skin or the like. Rubberized material involved the drawback of being too heavy in weight. 15 On the other hand animal products such as goldbeater's skin were too sensitive against friction, too little resistive to ripping and (unless a considerable number of layers were used) not sufficiently gastight. For all these 20 reasons animal products such as skins and intestines had to be employed in a number of superposed layers, this way of proceeding however leading to an enormous consumption of material so that it proved impossible to 25 satisfy the demand.

All these drawbacks are obviated in a very simple and yet effective manner by using the mass forming the object of the present invention, such mass substantially consisting 30 of a mixture of glue, preferably bone-glue, or some other material having the principal characteristics of glue, and a substance or substances adapted to render the glue as well as the fabric, skin or other material, to which 35 it is applied, elastic and gastight, amongst such substances being oils, such as Turkey red oil or other oils having similar properties, glycerin and the like. Of substances adapted to replace ordinary or bone-glue we merely 40 mention as the most conspicuous isinglass, casein and gelatine.

The preferred mixture consists of 100 parts water, 10 parts gelatine, 10 parts Turkey red oil or turcon oil, this being a substitute for 45 the former, and 5 parts glycerine, 0.25 parts bichromate of potash or formaldehyde being present, if desired, in order to render the mixture highly waterproof.

By aid of this mixture a balloon envelope 50 material is obtained which is superior to all

existing materials, either of vegetable or animal origin inasmuch as it presents the advantages offered by the skins and intestines before all others, and yet avoids their drawbacks enumerated above.

The novel mixture may either be used as an impregnating mass for cotton fabric, percale or other textile material and, if used in this way, renders the fabric absolutely gas- and watertight, without unduly increasing its weight, its elasticity being so great as to enable it to withstand all stresses acting on the envelope.

The mass having a composition as described above is then preferably spread on the stretched fabric in such manner that the spreading machine is at first adjusted for applying only a very thin coating to the fabric, the subsequent coatings from the third or fourth upwards being made thicker. Instead of spreading the impregnating mass on the fabric, we may dip the fabric into the mass, the fabric being thereafter freed from the impregnating mass in excess by causing it to pass between a pair of cylinders. In this case as well, we prefer starting with a slight impregnation. In order to render the product thus obtained waterproof, its inner and outer surfaces preferably receive a coating of good balloon varnish.

(The foregoing was disclosed in applicants' co-pending application Ser. No. 495,934. It was required by the Patent Office to be divided out of that application by office action of January 18, 1924. Applicants have inserted this matter in this instant application rather than filing a division application and thus avoiding a multiplicity of applications which has been condemned by the courts—see *Norden v. Spaulding* C. D. 1905 p. 588. Moreover this subject matter is specifically disclosed in German Patent No. 307,755 which is supplementary or additional to German Patent No. 303,809.)

It will be understood that without departing from the spirit of this invention, glycerine and Turkey red oil could be omitted from the mixture hereinbefore set forth.

It is to be distinctly understood that applicants do not confine their invention to the

55

60

65

70

75

80

85

90

95

100

specific use of glycerine or Turkey red oil as set forth in the specification. Oils, non-soluble fatty acids and the like can be employed in lieu thereof. The essence of the invention 5 resides in a mixture of animal glue and a substance, or substances, adapted to render the glue elastic, a list of such substances having been hereinbefore set forth.

We claim:

10 A composition for impregnating balloon fabrics adapted to be applied to cotton fabrics and the like, and when so applied and dried, to render such fabrics gas-tight without unduly increasing the weight thereof, and without substantially reducing their flexibility or elasticity, such composition comprising a glue-like substance, Turkey red oil approximately equal in quantity to the glue-like substance, approximately ten times as much 15 water as the glue-like substance and approximately half as much glycerine as the glue-like substance.

In testimony whereof we hereunto affix our signatures.

25 ERICH TRENCKMANN.  
BRUNO TRENCKMANN.

30

35

40

45

50

55

60

65